

**1****3,672,895****VACUUM TREATMENT OF COATED, DIRECT-POSITIVE, SILVER HALIDE ELEMENTS**

Richard Karl Kurz, Rochester, N.Y., assignor to Eastman Kodak Company, Rochester, N.Y.  
No Drawing. Filed Mar. 25, 1970, Ser. No. 22,697  
Int. Cl. G03c 5/24

U.S. Cl. 96—64

6 Claims

**ABSTRACT OF THE DISCLOSURE**

This invention relates to processes for improving the photographic properties of fogged, direct-positive, silver halide emulsions. In one aspect, coated, direct-positive emulsions are subjected to a vacuum treatment whereby the maximum density stability is improved upon aging. The  $D_{max}$  stability is highly improved in preferred embodiments when electron-acceptor compounds or desensitizers are present in the emulsion.

This invention relates to improved silver halide emulsions and methods of treating coated, direct-positive, silver halide emulsions to improve the photographic properties thereof. In one aspect, this invention relates to a process of subjecting coated silver halide emulsions or silver halide emulsion layers to a vacuum to stabilize the photographic properties; in one instance, the maximum density of fogged silver halide emulsions is stabilized upon aging, especially in fogged direct-positive emulsions containing densitizer compounds or electron acceptors.

It is known in the art to use various chemical addenda to stabilize the properties of silver halide emulsions upon aging. In certain instances, halide ions have been used to stabilize photographic properties such as sensitivity of silver halide emulsions. In other instances, it has become necessary to control temperature, humidity and the like carefully during shipping and storage to minimize the loss of image density and the increases in background fog. In some instances, formaldehyde has been added to the coated silver halide emulsions to improve aging properties or, in still other systems, the coated emulsions have been desiccated to improve properties. However, it is desirable to provide improved simple techniques for stabilizing the photographic properties of silver halide emulsions, especially fogged, direct-positive, silver halide emulsions which are not as easily stabilized as negative emulsions.

I have now found that the stability of fogged, direct-positive silver halide emulsions can be improved when the coated emulsions or emulsion layers are subjected to a vacuum of at least 1 torr and preferably of at least 0.1 torr. The coated layer is subjected to the vacuum for a period of at least 1 minute and preferably at least 5 minutes. Very good improvements in stability of the emulsion are obtained by this procedure, especially with fogged, direct-positive, silver halide emulsions containing electron acceptors.

While it is known that vacuum treatment of negative emulsions containing certain compounds will reduce desensitization of the emulsion, i.e., loss of photographic speed, or that in other instances it will increase speed of negative emulsions, it is quite unexpected that the maximum density stability of fogged, direct-positive emulsions would be affected by vacuum treatment of the emulsion as discovered in this invention.

In one preferred embodiment, the silver halide emulsions treated in accordance with this invention contain an electron-accepting compound which has an anodic polarographic halfwave potential and a cathodic half-wave potential which, when added together, give a positive sum.

**2**

In another preferred embodiment of this invention, the fogged, direct-positive emulsions treated in accordance with this invention are reduction and gold fogged.

In another embodiment of this invention, the fogged silver halide elements which comprise at least one layer of a fogged, direct-positive emulsion are subjected to an effective vacuum at the surface of said element of at least 1 torr and preferably at least 0.1 torr for at least 1 minute and preferably at least 5 minutes.

- 10 The direct-positive silver halide compositions which can be improved by the present process can be generally classified as blue-sensitive-direct-positive silver halide compositions. It is understood that "blue-sensitive" means that the direct-positive compositions will provide a reversal image when exposed with light in the 350- to 500-millimicron range of the electromagnetic spectrum and then developed. The silver halide compositions can also be spectrally sensitized so as to form reversal images when exposed in other regions of the spectrum such as 15 20 in the green and red regions. However, they all have the property of being capable of forming a reversal image when exposed with light in the blue region of the visible spectrum.

Typical direct-positive silver halide compositions which 25 can be treated in accordance with the present invention include:

- (1) Emulsions containing fogged silver halide grains which have internal centers for the deposition of photo- 30 lytic silver such as those generally disclosed in Berriman, U.S. Pat. 3,367,778 issued Feb. 6, 1968, including emulsions comprising grains which have centers which promote the deposition of silver which are either sufficiently small or sufficiently buried within the crystal as to be not accessible to initiate surface development to a visible 35 image. Silver halide grains of this latter type can be provided by (a) using a very low concentrations of sensitizing agent throughout the precipitation, (b) adding the sensitizing agent to the precipitation medium during the initial part of the precipitation and (c) reducing part of 40 the silver nitrate used in the initial portion of the precipitation, etc.

(2) Emulsions which contain silver halide grains which are uniformly fogged to specific levels and contain 45 electron-accepting compounds adjacent the grains, as described in Illingsworth, U.S. Ser. No. 619,948 filed Mar. 2, 1967, now Pat. No. 3,501,305.

(3) Emulsions comprising fogged regular grains which contain an electron-accepting compound of desensitizer 50 adjacent the grains, as described in Illingsworth, U.S. Ser. No. 619,909 filed Mar. 2, 1967, now Pat. No. 3,501,306.

(4) Emulsions comprising monodispersed grains which have been reduction and gold fogged, as described in 55 Illingsworth, U.S. Ser. No. 619,936 filed Mar. 2, 1967, now Pat. No. 3,501,307.

(5) Emulsions similar to the above which provide a reversal image when exposed to blue light.

The silver halides employed in the preparation of the 60 photographic compositions described herein include any of the photographic silver halides as exemplified by silver bromide, silver chloride, silver chlorobromide, silver bromoiodide, silver chlorobromide, and the like. Silver halide grains having a mean grain diameter, i.e., an 65 average grain size in the range of about .01 to about 2 microns, preferably about .02 to about 1 micron, give particularly good results in reversal systems. The silver halide grains can be any suitable shape such as cubic or octahedral, but they are preferably cubic, and more preferably cubic-regular. The preferred photographic silver halide emulsions comprise at least 50 mole percent bromide, the most preferred emulsions being silver

bromoiodide emulsions, particularly those containing less than about 10 mole percent iodide. The photographic silver halides can be coated at silver coverages in the range of about 50 to about 500 milligrams of silver per square foot of support.

The direct-positive photographic silver halide emulsions of this invention contain silver halide grains which are fogged. Fogging can be effected by chemically or physically treating the photographic silver halides by methods previously described in the prior art. Such fogging can be accomplished by various techniques such as chemical sensitization to fog, particularly good results being obtained with techniques of the type described by Antoine Hautot and Henri Saubener in *Science et Industries Photographiques*, vol. XXVIII, January 1957, pages 57-65. The silver halide grains can be fogged with the high-intensity light, reduction fogged with a reducing agent such as thiourea dioxide or stannous chloride or fogged with gold or noble metal compounds. Combinations of reduction fogging agents with gold compounds or compounds of another metal more electropositive than silver, e.g., rhodium, platinum or iridium, can be used in fogging the silver halide grains. The fogged silver halide grains in the direct-positive photographic emulsions of this invention give a density of at least 0.5 when developed without exposure for 5 minutes at 68° F. in Kodak DK-50 developer when a direct-positive emulsion containing such grains is coated at a coverage of 50 to about 500 mg. of silver per square foot of support.

The direct-positive photographic emulsions of this invention preferably comprise reduction and gold fogged silver halide grains, i.e., silver halide grains which are fogged with a combination of a reduction fogging agent and a gold fogging agent. Generally, about 0.0005 to about 0.06, preferably about 0.001 to about 0.03, milliequivalent of reduction fogging agent per mole of silver halide is employed in fogging the silver halide grains in certain embodiments of this invention. Examples of suitable reduction fogging agents which can be employed in the practice of this invention include hydrazine, phosphonium salts such as tetra(hydroxy methyl)phosphonium chloride, thiourea dioxide as disclosed in U.S. Pats. 3,062,651 by Hillson issued Nov. 6, 1962, and 2,983,609 by Allen et al. issued May 9, 1961, reducing agents such as the stannous salts, e.g., stannous chloride, as disclosed in U.S. Pat. 2,487,850 by Carroll issued Nov. 15, 1939, polyamines such as diethylene triamine as disclosed in U.S. Pat. 2,519,698 by Lowe et al. issued Aug. 15, 1950, polyamines such as spermine as disclosed in U.S. Pat. 2,521,925 by Lowe et al. issued Sept. 12, 1950, bis(β-aminoethyl) sulfide and its water-soluble salts as disclosed in U.S. Pat. 2,521,926 by Lowe et al. issued Sept. 12, 1950, and the like.

The gold fogging agents which can be employed in practicing this invention can be any gold salt suitable for use in fogging photographic silver halide grains and includes the gold salts disclosed in U.S. Pats. 2,399,083 by Waller et al. issued Apr. 23, 1946, and 2,642,361 by Damschroder et al. issued June 16, 1953. Specific examples of gold fogging agents are potassium chloroaurite, potassium aurithiocyanate, potassium chloroaurate, auric trichloride, 2-aurosulfobenzothiazole metho chloride, and the like. The concentration of gold fogging agent employed in the practice of this invention is subject to variation, but is generally in the range of about 0.001 to about 0.01 millimole per mole of silver halide. Potassium chloroaurate is a preferred gold fogging agent and is often used at concentrations of less than about 5 mg. per mole of silver halide and preferably at concentrations in the range of about 0.5 to about 4 mg. per mole of silver halide.

Preferably, the direct-positive emulsions used in this invention contain electron-accepting compounds, often referred to as desensitizers or electron traps, which are generally compounds having an anodic polarographic

halfwave potential and a cathodic polarographic potential which, when added together, give a positive sum. Typical useful electron-accepting compounds, along with methods of determining the polarographic potentials, are disclosed in the above-mentioned applications on direct-positive emulsions, as well as in Illingsworth et al., U.S. Ser. No. 609,761 filed Jan. 17, 1967. An especially useful class of electron acceptors which can be used in the direct-positive photographic silver halide emulsions and processes of this invention are cyanine dyes such as the imidazo[4,5-b] quinoxaline dyes. Dyes of this class are described in Brooker and Van Lare, Belgian Pat. 660,253 issued Mar. 15, 1965. In these dyes, the imidazo[4,5-b] quinoxaline nucleus is attached, through the 2-carbon atom thereof, to the methine chain.

In highly preferred embodiments of this invention, good improvements in  $D_{max}$  stability are obtained when the direct-positive emulsions contain electron acceptors having the above polarographic halfwave potentials, and are further characterized as those which spectrally sensitize the emulsion to radiation having a wave length longer than about 480 mμ so that the ratio of relative minus blue speed to relative blue speed is greater than 7. Electron acceptors of this type are disclosed in Illingsworth et al., U.S. Ser. No. 609,761 filed Jan. 17, 1967.

The vacuum treatment can be achieved by any method generally used for this purpose. In a typical embodiment, the coated element is located in a chamber and the chamber is pumped down to obtain a vacuum of at least 1 torr and preferably at least 0.1 torr for at least 1 minute and preferably at least 5 minutes. It is understood that this vacuum must be obtained at the surface of the coated element. Therefore, when rolls of film are treated, it may take considerably longer treatment periods to achieve this vacuum at the center of the roll, depending on the width of the film roll, tightness of winding, etc. Generally longer pumping periods will be necessary with large elements or rolls of the coated element due to outgassing. However, improved results are generally obtained as long as the respective portions of the element are directly subject to the vacuum for the indicated time periods.

If desired, the vacuum chamber can be purged with inert gases, such as nitrogen, after initial pumpdown. In certain instances, it is also desirable to rehumidify the coated films when very lengthy vacuum periods are used to stabilize the coated film.

After the specified pumpdown period, the coated elements can be stored in inert gases, air or the like. In certain instances, they have even been stored in oxygen without the concomitant degradation in  $D_{max}$  which usually occurs when the film is subjected to an oxygen environment.

The direct-positive emulsions of this invention also can contain compounds referred to as halogen-accepting or halogen-conducting compounds, especially if the halide of emulsion is predominantly chloride. Useful compounds of this type are generally characterized by an anodic polarographic potential less than 0.85 and a cathodic polarographic potential which is more negative than -1.0. Highly preferred species of compounds of this type are merocyanine dyes having the above halfwave potentials. Typical compounds of this type, along with methods of determining the polarographic potential, are disclosed in the above-mentioned applications on direct-positive emulsions as well as in Wise, U.S. Ser. No. 615,360 filed Feb. 13, 1967, now Patent No. 3,537,858.

The emulsions of this invention can also contain the hardeners, coating aids, surfactants, development modifiers, sensitizers, stabilizers, incorporated developer agents, binder vehicles and lubricants as disclosed in the art for direct-positive emulsions.

The invention can be further illustrated by the following examples of preferred embodiments thereof.

5

**EXAMPLE 1**

A reduction and gold fogged direct-positive silver bromoiodide (2.5 mole percent iodide) gelatin emulsion of the type described in Berriman, U.S. Pat. 3,367,778, is coated on a cellulose acetate film support which contains a layer of gelatin 175 mg./ft.<sup>2</sup> (Sample 1). The emulsion coverage is 120 mg. of silver and 178 mg. of gelatin/ft.<sup>2</sup> with a gelatin layer overcoat at 82.5 mg./ft.<sup>2</sup>.

The following additional coatings are prepared:

Sample 2 is like Sample 1 with 0.5% formaldehyde based on the total gelatin (or 2 g. formaldehyde/Ag mole) added to the emulsion;

to standard film boxes and held for 6 hours before being exposed and processed as a group. Exposure is for 1 sec. to a 500 w. 3000° K. light source in an Eastman 1B sensitometer and development is for 6 minutes in an Elon-hydroquinone developer with subsequent fixings, washing and drying. On comparing these coatings to a set of coatings which have been exposed and processed in the same manner soon after coating, there is found to be substantially no change in  $D_{max}$  on incubation at 70°-50% RH.

The effects of the 7-day incubation conditions on the  $D_{max}$  of the coatings are shown in Table 1. The numbers in this table are the obtained maximum density values.

TABLE I

| Sample | Pumpdown   |      |             |      |        |  |                         |                         |                         |                         |
|--------|------------|------|-------------|------|--------|--|-------------------------|-------------------------|-------------------------|-------------------------|
|        | 70°-50% RH |      | 120°-50% RH |      | Vacuum |  | Dry N <sub>2</sub> 120° | Wet N <sub>2</sub> 120° | Dry O <sub>2</sub> 120° | Wet O <sub>2</sub> 120° |
|        | 70°        | 120° | 70°         | 120° |        |  |                         |                         |                         |                         |
| 1----- | 2.20       |      | 2.01        | 2.28 | 2.27   |  | 2.27                    | 2.21                    | 2.14                    | 2.09                    |
| 2----- | 2.09       |      | 1.96        | 2.10 | 2.19   |  | 2.16                    | 2.22                    | 2.10                    | 2.11                    |
| 3----- | 1.97       |      | 0.78        | 1.99 | 1.88   |  | 1.88                    | 1.83                    | 1.68                    | 1.65                    |
| 4----- | 1.87       |      | 0.85        | 1.90 | 1.97   |  | 1.90                    | 1.88                    | 1.82                    | 1.76                    |

Sample 3 is like Sample 1 with a phenyl-imidazoquin-oxaline-indolo carbocyanine dye (Dye I) of the type described in Brooker and Van Lare, U.S. Ser. No. 609,791, new Pat. No. 3,431,111, added to the emulsion at 650 mg./Ag mole;

Sample 4 is like Sample 1 with the combination of formaldehyde and Dye I added at the concentrations above.

The incubation properties of Samples 1-4 are evaluated for 7-day incubations under the following different incubation conditions:

70°-50% RH air  
 70°-vacuum  
 120°-vacuum  
 120°-“dry” nitrogen  
 120°-“wet” nitrogen  
 120°-50% RH air  
 120°-“dry” oxygen  
 120°-“wet” oxygen

The film incubations, with the exception of the 70°-50% air incubations, are carried out in stainless-steel cylindrical bombs approximately 14 in. long x 2 1/8 in. diameter (volume=0.03 cu. ft.). The samples incubated at 70°-50% RH in air are stored in a standard film box. The strips of the four films stored in vacuum, nitrogen or oxygen are placed in the bombs as a group and pumped down in about 25 minutes to less than  $5 \times 10^{-2}$  torr. After being pumped down once, the samples are twice purged with the appropriate gas, and re-evacuated to less than  $5 \times 10^{-2}$  torr. in 3 min., finally being stored in vacuum, or in nitrogen or oxygen at +10 p.s.i. gauge pressure. The strips stored at 120°-50% RH in air are not pumped down but are sealed without further treatment in a stainless-steel bomb under ambient room conditions. The "dry" gases are conditioned by passing them through a silica gel column. The "wet" gases are conditioned to an unknown relative humidity by bubbling them through a saturated aqueous  $\text{Pb}(\text{NO}_3)_2$  solution which at 20° C. imparts a 98% RH to the atmosphere above the solution at equilibrium.

At the end of the 7-day incubations, the bombs held at 120° are allowed to cool overnight to room temperature and are then opened to the air. The samples are removed

$D_{\max}$  losses of the films incubated in air at 120°-50% are substantial relative to losses under all the other conditions. The two films, Sample 3 and Sample 4, containing Dye I show major  $D_{\max}$  losses in air at 120°-50% RH. The distinctive treatment of the films stored at 120°-50% RH in air is that they are *not* pumped down in vacuum. The pumped-down films, even those that are stored in pure oxygen at 120°, are relatively stable.

Similar improvements are observed when the electron-accepting compound, Dye I, is replaced in Samples 3 and 4 with

35 1,1'-dimethyl-2,2'-diphenyl-3,3'-indolocarbocyanine bromide; 1,1'-dimethyl-2,2',8-triphenyl-3,3'-indolocarbocyanine perchlorate; 2,2'-di-p-methoxyphenyl-1,1'-dimethyl-3,3'-indolocarbocyanine bromide; 40 1,1',3,3'-tetraethylimidazo-[4,5-b]quinoxalinocarbocyanine chloride; or 5,5'-dichloro-3,3'-diethyl-6,6'-dinitrothiacarbocyanine iodide.

### EXAMPLE 2

To show that the stabilization seen in Table 1 is the result of pumpdown or evacuation and not the result of a nitrogen or oxygen atmosphere, sets of the coatings used in Example 1 are incubated in nitrogen and oxygen atmospheres with no evacuation. The procedure is the same as in Example 1 with the following 7-day incubation conditions:

|                          | Evacuated | Purged |
|--------------------------|-----------|--------|
| 70°-50% RH air.....      | -         | -      |
| 120°-vacuum.....         | +         | -      |
| 120°-“dry” nitrogen..... | +         | -      |
| Do.....                  | -         | +      |
| 120°-Air.....            | +         | -      |
| Do.....                  | -         | +      |
| 120°-“dry” oxygen.....   | +         | -      |
| Do.....                  | -         | +      |

The samples which are purged are placed in the bombs and the appropriate gas is passed through the bombs for 5 minutes, no evacuation being employed, after which the bombs with nitrogen and oxygen are pressurized to +10 p.s.i. gauge pressure.

The  $D_{max}$  stabilization of the films by vacuum treatment is confirmed by the results in Table 2. The actual  $D_{max}$  values are given for each treatment.

TABLE 2

| Sample | 120° air      |       |               | 120° dry N <sub>2</sub> |       |               | 120° dry O <sub>2</sub> |               |  |
|--------|---------------|-------|---------------|-------------------------|-------|---------------|-------------------------|---------------|--|
|        | 70°<br>50% RH | Purge | Pump-<br>down | 120°<br>vacuum          | Purge | Pump-<br>down | Purge                   | Pump-<br>down |  |
| 1      | 2.21          | 1.83  | 2.15          | 2.21                    | 2.08  | 2.30          | 1.78                    | 2.0           |  |
| 2      | 2.09          | 1.90  | 2.21          | 2.21                    | 2.08  | 2.19          | 1.82                    | 2.1           |  |
| 3      | 1.96          | 0.80  | 1.74          | 1.87                    | 1.36  | 1.79          | 0.60                    | 1.4           |  |
| 4      | 1.81          | 0.83  | 1.81          | 1.84                    | 1.38  | 1.79          | 0.66                    | 1.7           |  |

The stabilizing effect of the evacuation on the  $D_{max}$  of all four films incubated at 120° in nitrogen, air or oxygen is consistently demonstrated. The stabilizing effect of formaldehyde is also apparent in that both the non-dyed control (Sample 1) and the dyed film (Sample 3) show greater  $D_{max}$  losses under all conditions than their formaldehyde-containing counterparts, Sample 2 and Sample 4, respectively.

#### EXAMPLE 3

The vacuum treatment can also be used with spools of film. Four rolls (100 ft. x 35 mm.) of an emulsion coating similar to Sample 4, i.e., containing Dye I at 570 mg./Ag mole and formaldehyde, are placed in a vacuum chamber and evacuated for 23 hours to a pressure of ca.  $5 \times 10^{-2}$  torr. The chamber is returned to ambient room conditions (70°-50% RH), then re-evacuated for 1 hour to ca.  $5 \times 10^{-2}$  torr and finally returned to ambient room conditions. The rolls of film are placed back in a metal container and are held for 4 hours prior to being incubated. One of the four rolls is kept for an additional 24 hours at room conditions before being incubated. These rolls and three control rolls, treated and incubated for 7 days, as listed in Table 3, are compared in the experiment. Following the incubations, the rolls are cooled to room temperature, are removed from the sealed bags and are conditioned for 3 hours at ambient room conditions before being exposed. Duplicate strips taken from the outside, middle and core areas of the rolls are exposed and processed as a group. The average gain or loss in  $D_{max}$  of the samples taken from the three areas of the rolls are listed in Table 3 with the  $D_{max}$  of the film kept at 70°-50% RH with no vacuum treatment (Roll 1) taken as the reference ( $D_{max}=2.50$ ).

TABLE 3

| Roll No. | Conditions                                                            | Change in $D_{max}$ after 1 wk. incubation of rolls |        |      |
|----------|-----------------------------------------------------------------------|-----------------------------------------------------|--------|------|
|          |                                                                       | Outside                                             | Middle | Core |
| 1        | 70°-50% RH air—no pumpdown                                            | 0                                                   | 0      | 0    |
| 2        | 70°-50% RH air—with pumpdown                                          | +.04                                                | +.01   | +.02 |
| 3        | 120°-50% RH air—no pumpdown                                           | -.45                                                | -.38   | -.45 |
| 4        | 120°-50% RH air—with pumpdown                                         | -.15                                                | -.15   | -.02 |
| 5        | 120° oxygen <sup>1</sup> —no pumpdown                                 | -.55                                                | -.63   | -.63 |
| 6        | 120° oxygen <sup>1</sup> —with pumpdown                               | -.12                                                | -.11   | +.02 |
| 7        | 120°-50% air—with pumpdown and 24-hour conditioning before incubation | -.13                                                | -.04   | +.02 |

<sup>1</sup> The incubations in an oxygen atmosphere are obtained by purging the foil-lined incubation bag containing the roll with oxygen for 5 minutes immediately before sealing the bag.

The vacuum treatment is generally effective in stabilizing the outside, middle and core areas of the rolls. The vacuum treatment itself of Roll 2 held under room-temperature conditions has little effect on the  $D_{max}$ . Incubation in air at 120° (Roll 3) with no vacuum treatment simulating aging conditions produces an average loss in  $D_{max}$  of 0.43, while incubation of the vacuum-treated film (Roll 4) under the same conditions produces an average loss in  $D_{max}$  of only 0.11. Incubations in oxygen at 120° produce an average 0.60  $D_{max}$  loss for the film with no vacuum treatment (Roll 5), while the vacuum-treated film (Roll 6) has an average  $D_{max}$  loss of only about 0.07. The vacuum-treated film which is stored 24 hours under room conditions before 120° incubation in air (Roll 7) has an average  $D_{max}$  loss of 0.05.

#### EXAMPLE 4

Among the many possible explanations offered for the stabilization conferred on the direct-positive films by vacuum treatment are the degassing and dehumidification of the film by the vacuum. An attempt to separate the degassing and dehumidification effects on stability is made

by comparing desiccated strips of Sample 3 to strips of the same sample subjected to mild degassing vacuum for short times (which would not substantially dehumidify the film).

Desiccation is for 76 hours over  $P_2O_5$  followed by 1 week's 120°-50% RH incubation of the desiccated film in air and 1 week of keeping of another sample of desiccated film at 70°-50% RH to observe the effect of desiccation itself on the film. The effects of low vacuum on the stability are evaluated by placing duplicate 12 in. x 35 mm. strips of Sample 3 in the stainless-steel bombs (described previously) and, with a mechanical vacuum pump which produces at  $10^{-1}$  torr vacuum, pumping on the strips for 1, 10 and 30 minutes to a  $10^{-1}$  torr pressure followed in each case by two successive cycles of release of the vacuum and 1-min. re-evacuation for a total of 3, 12 and 32 minutes. The several vacuum-treated strips are incubated separately at 120° in air for 1 week and compared with non-evacuated control strips similarly incubated. The  $\Delta D_{max}$  values for these films are listed in Table 4 in which the  $D_{max}=1.88$  of the room-incubated control is used as the reference  $D_{max}$  for calculating the  $\Delta D_{max}$  values of the other incubated samples.

TABLE 4

| Condition:                                    | Change in $D_{max}$            |                                                      |
|-----------------------------------------------|--------------------------------|------------------------------------------------------|
|                                               | Control, 1 wk. inc. 70°-50% RH | Control 76 hours' desiccation, 1 wk. inc. 70°-50% RH |
| Control, 1 wk. inc. 120°-50% RH               | —                              | +.01                                                 |
| 76 hours' desiccation, 1 wk. inc. 120°-50% RH | —.60                           | —                                                    |
| 3 min. pumpdown, 1 wk. inc. 120°-50% RH       | —.33                           | —.56                                                 |
| 12 min. pumpdown, 1 wk. inc. 120°-50% RH      | —.31                           | —                                                    |
| 32 min. pumpdown, 1 wk. inc. 120°-50% RH      | —.27                           | —                                                    |

Desiccation itself for 76 hours has little effect on film  $D_{max}$  and has no significant stabilizing effect on the  $D_{max}$  of the incubated samples relative to the incubated control which shows a  $D_{max}$  loss=0.60. The low vacuum ( $10^{-1}$  torr) treatments of the film produce a definite stabilization which reduces the  $D_{max}$  loss on incubation from the 0.60 value of the control to about 0.30 for the experiments. The fact that these short, low-vacuum treatments produce a significant stabilization, whereas extended desiccation over  $P_2O_5$  does not alter the incubation stability of the film, indicates that stabilization does not occur via a moisture removal effect.

Although the invention has been described in considerable detail with particular reference to certain preferred embodiments thereof, variations and modifications can be effected within the spirit and scope of the invention.

I claim:

1. A process for treating a fogged, direct-positive, silver halide element comprising subjecting said element, which comprises at least one layer containing a fogged, direct-positive, silver halide emulsion, to a vacuum of at least 1 torr at the surface of said silver halide element for a time sufficient to improve  $D_{max}$  stability of said silver halide emulsion.
2. A process according to claim 1 wherein said fogged, silver halide emulsion is reduction and gold fogged.
3. A process according to claim 1 wherein said fogged, direct-positive, silver halide emulsion contains an electron-accepting compound which has an anodic polarographic halfwave potential and a cathodic halfwave potential which, when added together, give a positive sum.
4. A process according to claim 1 wherein said fogged, direct-positive, silver halide emulsion contains an electron-accepting compound which is characterized as one which spectrally sensitizes the emulsion to radiation having a wave length longer than about 480 m $\mu$  so that the ratio of relative minus blue speed to relative blue speed is greater than 7.

3,672,895

9

5. A process according to claim 1 wherein a vacuum of at least 0.1 torr is maintained for at least 5 minutes.

6. A process according to claim 1 wherein said element is subjected to said vacuum shortly after coating the emulsion and before exposure.

10

FOREIGN PATENTS

|         |         |               |       |       |
|---------|---------|---------------|-------|-------|
| 281,700 | 12/1927 | Great Britain | ----- | 34—16 |
| 6,735   | 12/1899 | Great Britain | ----- | 34—16 |
| 672,156 | 2/1939  | Germany       | ----- | 34—16 |

5

NORMAN G. TORCHIN, Primary Examiner

W. H. LOUIE, JR., Assistant Examiner

U.S. Cl. X.R.

References Cited

UNITED STATES PATENTS

|           |        |                |       |         |    |               |
|-----------|--------|----------------|-------|---------|----|---------------|
| 1,861,918 | 6/1932 | Hickman        | ----- | 34—16 X | 10 | 34—16; 117—34 |
| 2,115,747 | 5/1938 | Rafton         | ----- | 34—16   |    |               |
| 1,180,255 | 4/1916 | Cossitt et al. | ----- | 34—16 X |    |               |